

## UNITED STATES PATENT OFFICE

WILLIAM ROY MOORHOUSE, OF NEW YORK, N. Y., ASSIGNOR TO NATIONAL ANILINE & CHEMICAL COMPANY, INC., OF NEW YORK, N. Y., A CORPORATION OF NEW YORK

## DYEING PROCESS

No Drawing. Application filed February 25, 1929. Serial No. 342,674.

This invention relates to the dyeing of textile fabrics by means of vat dyes.

There are three principal methods generally employed for dyeing cotton and rayon piece goods with vat dyes, namely: (1) working the material to be dyed in a bath of the reduced dyestuff; (2) padding the material to be dyed with the reduced dyestuff, and then developing the color by working the padded material in a reducing bath; and (3) padding the material to be dyed with the unreduced dyestuff, and then working the padded material in a reducing bath, or "jigging" it.

The dyeing of textile fabrics and fibres with vat dyes by the third method, called the "pad and jig" method or the "pigment padding" method is disclosed by Schlegel in United States Patents Nos. 893,384 and 1,185,943. According to this process, the material to be dyed with the vat dyestuff (e. g. cotton fabric, yarn, and the like) is padded or printed with a paste which contains the vat dyestuff in the unreduced form (pigment form), water, and a suitable thickener. It is then rolled up, either with or without drying, and transferred to the jigger where it is treated with a solution or suspension of an alkaline reducing agent (such as, for example, alkaline hydrosulfite) in order to develop the color on the fibre. The material is then finished in any suitable manner; e. g. by passing it through oxidizing and soaping baths.

The present invention relates to improvements in the process of dyeing cotton and regenerated cellulose (rayon) piece goods and yarn by the said pad and jig method, and is especially concerned with improvements in the padding process and the padding liquor.

One of the objects of the present invention is the provision of a padding liquor which produces dyeings of improved strength and brightness of shade.

Another object of the invention is the incorporation into a padding liquor of a substance which increases the rapidity with which the vat dyestuff contained in the liquor is developed on the fibre on the jig.

Another object of the invention is the in-

corporation into a padding paste or liquor of a substance which enhances the smoothness of the paste and permits it to be more readily strained.

These and other objects of the invention will be apparent from a consideration of the following disclosure which is given for the purpose of illustrating the invention.

According to the present invention, the material to be dyed with a vat dyestuff is padded with a padding liquor which contains the vat dyestuff in the unreduced form and an alkali metal salt whose aqueous solutions react alkaline. The expression "vat dyestuff in the unreduced form", as used in this description and in the claims, denotes the vat dyestuff as distinguished from its leuco-derivatives.

It has been found, according to the present invention, if in dyeing by the pad and jig method the material be padded with a padding liquor which contains a suitable alkali-metal salt whose aqueous solutions react alkaline, that the dyeings obtained are of an improved quality, as indicated by the increased strength and brightness of shade of the dyeings obtained with said liquor as compared with dyeings made under identical conditions with a similar padding liquor which, however, does not contain said alkali-metal salt.

It has furthermore been found, according to the present invention, that if into the padding liquor containing the vat dyestuff in the unreduced form there is incorporated a suitable alkali-metal salt whose aqueous solutions react alkaline, the working qualities of the padding liquor or paste are improved, as evidenced by the facts that the paste is smoother and can be strained more readily. In addition, when material padded with a padding liquor which contains such an alkali-metal salt is subjected to the action of the reducing bath on the jig, the color is developed on the fibre with greater rapidity than when said salt is not present.

In carrying out the process according to a preferred method of procedure, a padding liquor is prepared containing a mixture of a suitable vat dyestuff in the unreduced form, a suitable alkali-metal salt, water, and a suit-

able gum, adhesive, or thickener. The mixture is strained through a cloth of fine mesh, and the material to be dyed (such as, cotton, linen, or rayon piece goods or yarn) is padded 5 or printed with the resulting liquor. The padded or printed cloth is then treated in the usual manner on the jig or in a suitable reducing bath (such as, an alkaline hydrosulfite bath) and subsequently finished in the cus- 10 tomary way.

In preparing the padding liquor, the vat dyestuff employed, which may be, for example, an anthraquinone vat dye or an indigo vat dye, is preferably used in the paste 15 form.

Among the anthraquinone vat dyestuffs which are particularly useful in connection with the invention are the anthraquinone azine vat dyes; such as, indanthrone, flavanthrone, halogenated indanthrones, etc. 20

Among the alkali-metal salts suitable for incorporation into the padding liquor, there may be mentioned, by way of example, the alkaline alkali-metal salts of phosphoric acid, silicic acid, carbonic acid, hydrogen 25

sulfide, and the like (such as, disodium and trisodium phosphates, sodium silicate, sodium carbonate, potassium carbonate, sodium sulfide, ammonium sulfide, etc.), the alkali-metal salts of the higher fatty acids 30

(such as, sodium stearate, sodium oleate, sodium palmitate, or their corresponding potassium salts), and the alkali-metal salts of sulfonated fatty acids (such as, the sodium or ammonium salts of sulfonated castor oil); 35

and it will be understood that where in the claims the expression "an alkali-metal salt whose aqueous solutions react alkaline" is used, it meant to include the above salts and their equivalent salts.

The invention will be described in connection with the following examples which are given for illustrative purposes only, it not being intended to limit the procedure to the details given.

*Example 1.*—A padding liquor is prepared containing the following ingredients in the following approximate amounts:

|                                                                   |          |
|-------------------------------------------------------------------|----------|
| Carbanthrene blue GCD double<br>paste (Colour index No. 1113) ... | 30 gms.  |
| Trisodium phosphate-----                                          | 3 gms.   |
| Gum tragacanth-----                                               | 3.6 gms. |
| Gum arabic-----                                                   | 6.8 gms. |
| Water sufficient to make up volume<br>to approximately-----       | 1700 cc. |

For example, by mixing the dyestuff with the sodium phosphate, which is preferably in the form of a water solution, adding the gum arabic and gum tragacanth in the form of water solution, bringing the total volume up to the desired volume by addition of water, and straining the mixture through a cloth of fine mesh. Cotton piece goods is padded or printed with the liquor in a suitable manner known to the art (for example,

by passing the cloth between rolls through the padding liquor which is preferably at a temperature of about 120° F.), the padded or printed cloth is treated on the jig in an alkaline hydrosulfite bath, preferably maintained at a temperature of about 140°-160° F., wherein the color rapidly develops, and is then finished as usual.

The dyeings obtained are of an increased brightness and fullness of shade as compared with those obtained by the employment of a padding liquor containing no sodium phosphate but otherwise the same as that employed in this example.

*Example 2.*—Cotton cloth or yarn is padded in a padding liquor similar to the one described in Example 1, with the difference, however, that instead of the trisodium phosphate, the liquor contains 1.6 grams of sodium silicate. The padded cloth or yarn is subsequently treated as in Example 1.

*Example 3.*—The procedure and ingredients are the same as in Example 1, with the exception that 1.5 grams of Turkey red oil (consisting mainly of the sodium salt of sulfonated castor-oil) is employed instead of the trisodium phosphate of said example.

*Example 4.*—Cotton piece goods is padded in a padding liquor containing 30 grams of carbanthrene yellow G double paste (Colour index No. 1118) and 1.5 grams of a good grade of textile soap, such as Ivory soap, together with the gums and water in the proportions given in Example 1. The padded cloth is subsequently treated as above described.

*Example 5.*—The procedure and ingredients are the same as in Example 4, with the exception that 1.5 grams of sodium carbonate is employed instead of the soap of said example.

As pointed out above, the invention is not limited to the above specific examples, but broadly contemplates the incorporation into a padding liquor containing a vat dyestuff in unreduced form of a suitable alkali-metal salt whose aqueous solutions react alkaline.

The vat dyestuffs which are useful in the process are not limited to those given in the above examples, but other suitable vat dyestuffs may be employed; such as, other vat dyes of the anthraquinone series, including the indanthrones (particularly the halogenated indanthrones), flavanthrones, dibenzanthrones, etc. The quantities of dyestuff to be used will obviously vary with the particular dyestuff employed and with the shade and strength of color desired.

Instead of the alkali-metal salts used in the above examples, other suitable alkali-metal salts whose aqueous solutions react alkaline may be used, as above indicated; such as, alkali-metal salts of the higher fatty acids and of the sulfonated fatty oils and fatty acids, alkaline alkali-metal salts of the

polybasic inorganic acids, etc. And instead of a single alkali-metal salt, mixtures of two or more of said salts may be also employed. It will furthermore be evident that the salts 5 need not be pure but that technical products may be used, and such technical products may include mixtures of the alkali-metal salts of the fatty acids with some of the free fatty acid; e. g. commercial Turkey red oil.

10 The quantity of alkali-metal salt incorporated into the liquor will also vary within considerable limits depending upon the individual dyestuff, the individual salt, and the amount of dyestuff employed. Thus, for example, in making dyeings with carbanthrene blue GCD double paste and employing trisodium phosphate in the padding liquor, satisfactory results may be obtained with from about 3 to about 50 per cent by weight 15 of trisodium phosphate based on the weight of the double paste, although about 10 per cent of trisodium phosphate is preferred. It is to be noted, however, that within limits a relatively small quantity of alkali-metal salt 20 is preferred over a relatively large quantity; inasmuch as it has been found that instead of an improvement in the dyeings being effected, no improvement and even deleterious results are produced when too large a quantity 25 of alkali-metal salt is used. For example, the addition of too much alkali-metal salt often has been found to cause the paste to lump and the material to pad unevenly.

Various thickeners and adhesives (for example, glue, gelatin, and other mucilaginous materials), either alone or in admixture, may also be used instead of the gums described in the above examples; and the quantity to be employed may also vary, as will be evident. 30 The padding liquor is preferably prepared in the manner above described, but it will be evident that it may be prepared in a variety of ways, and that the order of mixing the ingredients may be suitably varied. While the 35 procedure and temperatures employed in the above examples are preferred, it will be evident that they also can be varied.

The process as described is an economical and rapid one. Dyeings of brighter and 40 fuller shades are obtained than by the prior pad and jig processes, and the development of the color on the jig is more rapid.

This application is a continuation in part of my copending application Serial No. 294,586, filed July 21, 1928, for "dyeing process", and contains subject matter specifically claimed in said application.

Having thus described my invention, what I claim and desire to secure by Letters Patent is:

1. In a process of dyeing with a vat dyestuff by the pad and jig method the improvement which comprises padding the material to be dyed with a padding liquor which 65 contains the vat dyestuff in the unreduced

form, a thickener and an alkali-metal salt whose aqueous solutions react alkaline.

2. In a process of dyeing with a vat dyestuff by the pad and jig method, the improvement which comprises padding the material to be dyed with a padding liquor which contains the vat dyestuff in the unreduced form and an alkaline alkali-metal salt of an inorganic polybasic acid.

3. In a process of dyeing with a vat dyestuff by the pad and jig method, the improvement which comprises padding the material to be dyed with a padding liquor which contains the vat dyestuff in the unreduced form and trisodium phosphate.

4. In a process of dyeing with a vat dyestuff by the pad and jig method, the improvement which comprises padding the material to be dyed with a padding liquor which contains the vat dyestuff in the unreduced form and an alkali-metal salt selected from the group consisting of trisodium phosphate, sodium carbonate and sodium silicate.

5. In a process of dyeing with a vat dyestuff by the pad and jig method, the improvement which comprises padding the material to be dyed with a padding liquor which contains the vat dyestuff in the unreduced form, a thickener, and an alkali-metal salt of a higher fatty acid.

6. In a process of dyeing with a vat dyestuff by the pad and jig method, the improvement which comprises padding the material to be dyed with a padding liquor which contains the vat dyestuff in the unreduced form, a thickener, and an alkali metal salt of a sulfonated higher fatty acid compound.

7. In the process of dyeing with a vat dyestuff by the pad and jig method, the improvement which comprises padding the material to be dyed with a padding liquor which contains the vat dyestuff in the unreduced form, a thickener, and Turkey-red oil.

8. In a process of dyeing with a vat dyestuff of the indigoid series by the pad and jig method, the improvement which comprises padding the material to be dyed with a padding liquor which contains the vat dyestuff of the indigoid series in the unreduced form, a thickener, and an alkali-metal salt whose aqueous solutions react alkaline.

9. In a process of dyeing with a vat dyestuff of the anthraquinone series by the pad and jig method, the improvement which comprises padding the material to be dyed with a padding liquor which contains the vat dyestuff of the anthraquinone series in the unreduced form, a thickener and an alkali-metal salt whose aqueous solutions react alkaline.

10. In a process of dyeing with an anthraquinone azine by the pad and jig method, the improvement which comprises padding the material to be dyed with a padding liquor which contains the anthraquinone azine in the unreduced form, a thickener, and an al-

kali-metal salt whose aqueous solutions react alkaline.

11. In a process of dyeing with an indanthrone by the pad and jig method the improvement which comprises padding the material to be dyed with a padding liquor which contains the indanthrone in the un-reduced form, and an alkali-metal salt whose aqueous solutions react alkaline.
12. In a process of dyeing with a chlor-indanthrone by the pad and jig method, the improvement which comprises padding the material to be dyed with a padding liquor which contains the chlorinated indanthrone in the un-reduced form and an alkali-metal salt whose aqueous solutions react alkaline.
13. In a process of dyeing with dichlor-indanthrone by the pad and jig method, the improvement which comprises padding the material to be dyed with a padding liquor which contains dichlor-indanthrone in the un-reduced form and trisodium phosphate.
14. A padding liquor comprising a vat dye-stuff substantially entirely in the un-reduced form, water, a thickener and an alkali-metal salt whose aqueous solutions react alkaline.
15. A padding liquor comprising a vat dye-stuff of the anthraquinone series substantially entirely in the un-reduced form, water, a thickener and an alkali-metal salt whose aqueous solutions react alkaline.
16. A padding liquor comprising an anthraquinone azine vat dyestuff substantially entirely in the un-reduced form, water, a thickener and an alkali-metal salt whose aqueous solutions react alkaline.
17. A padding liquor comprising an indanthrone substantially entirely in the un-reduced form, water and an alkali-metal salt whose aqueous solutions react alkaline.
18. A padding liquor comprising a vat dye-stuff of the indigoid series substantially entirely in the un-reduced form, water and an alkali-metal salt whose aqueous solutions react alkaline.
19. Material padded with the padding liquor of claim 14.
20. Material padded with the padding liquor of claim 15.
21. Material padded with the padding liquor of claim 16.
22. Material padded with the padding liquor of claim 17.
23. Material padded with the padding liquor of claim 18.

In testimony whereof I affix my signature.  
WILLIAM ROY MOORHOUSE.